

Patented Apr. 12, 1927.

1,624,599

# UNITED STATES PATENT OFFICE.

ROBERT W. HILTON, DECEASED, LATE OF CINCINNATI, OHIO; BY DANESI M. HILTON, EXECUTRIX, OF CINCINNATI, OHIO, ASSIGNOR TO THE KEMPER-THOMAS COMPANY, OF NORWOOD, OHIO, A CORPORATION OF OHIO.

## MANUFACTURE OF FIBER BOARD.

No Drawing.

Application filed November 1, 1923. Serial No. 672,208.

The invention relates to improvements in the manufacture of fiber board, and particularly to a fiber board which is especially adapted for use in the manufacture of printed signs.

The object of the invention is to produce a fiber board, suitable for the manufacture of signs which will be as nearly as possible impervious to water, so that the disintegrating effect of weathering, particularly of repeated wetting and drying will be reduced to a minimum.

A fiber board, made according to the process herein described will present an oil phase to inks used in printing thereon, so that the inks will have a greater affinity for the board than they would have for a fiber board of ordinary character and possessing such an oil phase and which are readily wetted by water.

Furthermore the printing surface of the treated board is smoother and freer from irregularities, thereby allowing the ink printed upon it to cover the surface more smoothly and to lie smoother than on ordinary board.

The essential step in this invention is to coat the fibers of a piece of board, with an insoluble metal soap, thereby protecting the fibers and making the board waterproof, excellent to print, smooth after calendering, and upon which the printed surface will be smooth and free from irregularities, as above stated.

The problem of getting the insoluble soap into the fiber may be solved in two ways, but preferably is done in the beating engine, when the paper is in the aqueous pulp stage. It may also be accomplished by treatment of the formed paper sheet, although this is more difficult and will probably require special apparatus in large commercial practice. Since each fiber must be coated with the material, to fully waterproof a web of paper, the process involves the chemical formation of the insoluble metal salt in the presence of the fibers.

The preferred process is carried out by adding to the beater, having a charge of paper stock and water therein, a soluble soap, of one of the fatty or other organic acids. Thus in one specific process there is added from one to three per cent of the soda

soap of fatty acids such as oleic, stearic, and palmitic acids, the same permitted to dissolve in the beater water so as to be intimately associated with the fibers in the beater charge.

Then are added the salts of some metals which form insoluble soaps of the organic acids employed in the first step, in sufficient quantity to re-act with all of the soluble soaps, and effect complete precipitation thereof, in the form of the insoluble soaps of said metals.

Thus in the specific process, of which the first step has been stated, there is formed and added to the beater a solution of the soluble salts of alumina, barium, lead, zinc, or other metals of the insoluble organic soap group sufficient to effect complete precipitation, so that the total quantity of metallic soaps produced will amount to from one to three per cent of the weight of the board that it is desired to produce.

One salt which has shown superior results in the process is lead acetate, which can easily be brought to solution in water, and is inexpensive.

The result of the precipitation of insoluble soap in the presence of the fiber, is that the individual fibers become coated with the same, and as the usual steps in the manufacture of paper are proceeded with, the resulting sheet will have its fibers thoroughly coated, and will exhibit the qualities above outlined.

Proceeding by the other process, which will be termed the saturation process, a pre-formed web of paper is used, and thoroughly impregnated with a solution of the soluble soap employed. To aid in this impregnation, and gain a thorough saturation of each fiber, it may be necessary to use pressure or a vacuum.

The saturated web is next treated with a solution of the metal salt, and again is thoroughly saturated, if necessary with pressure or vacuum, so as to gain a complete reaction, resulting as before in the precipitation of the insoluble soaps.

Finally, if necessary, the sodium salts left by the reaction, may be washed out of the web, by any desired method which will not disintegrate the web, and the web may then be calendered and dried.

For weatherproof signs, to be exposed to the elements, over long periods of time, the board produced by my process is excellent, and the improved printing surface it affords, 5 insures longer life for the printed design upon it.

This process should be distinguished from a sizing process, as it proceeds further than sizing, to the extent of the precipitation 10 upon the fibers of an insoluble body in dispersed or colloidal form.

Having thus described the process, what is claimed as new and desired to be secured by Letters Patent, is:—

The process of manufacturing weather 15 resistant fiber board, which consists in thoroughly mixing fiber pulp in an aqueous solution of soap and treating the pulp with lead acetate to precipitate insoluble lead soap in intimate admixture with said fiber, 20 the quantity of soap required being sufficient to provide approximately not over three per cent by weight of insoluble soap on the basis of the pulp used.

DANESI M. HILTON,  
*Executrix of the Estate of Robert W. Hilton, Deceased.*